

O. C. GILBERT AND E. W. ADAMS.  
METHOD OF WORKING METALS.  
APPLICATION FILED JUNE 24, 1919.

1,384,448.

Patented July 12, 1921.

Fig. 1.



Fig. 3.



Fig. 4.



Fig. 2.



Inventors:  
Oliver C. Gilbert.  
Edgar W. Adams.  
by *Robert* Atty.

# UNITED STATES PATENT OFFICE.

OLIVER C. GILBERT, OF NEW YORK, N. Y., AND EDGAR W. ADAMS, OF EAST ORANGE,  
NEW JERSEY; SAID ADAMS ASSIGNOR TO SAID GILBERT.

## METHOD OF WORKING METALS.

1,384,448.

Specification of Letters Patent. Patented July 12, 1921.

Application filed June 24, 1919. Serial No. 306,330.

To all whom it may concern:

Be it known that we, OLIVER C. GILBERT and EDGAR W. ADAMS, citizens of the United States, residing at New York, in the county 5 of New York and State of New York, and at East Orange, in the county of Essex and State of New Jersey, respectively, have invented certain new and useful Improvements in Methods of Working Metals, of which the 10 following is a full, clear, concise, and exact description.

This invention relates to a process for working metals and their alloys. More particularly, the invention relates to a process 15 of drawing metals whereby the drawn metal is given a shape, which cannot be obtained by the use of rolls and which cannot be feasibly attained with the use of a shaping die.

In the embodiment illustrated, the im- 20 proved process is shown as applied in the manufacture of tinsel formed of copper or other non-ferrous metals but it is to be understood the invention is not limited to this specific application or to the treatment of 25 metals having the susceptibilities of copper or other non-ferrous metals because the process herein may be employed to advantage for other purposes than the fabrication of tinsel and for the working of all metals 30 whether non-ferrous or not.

Figure 1 of the drawings illustrates dia- 35 grammatically a means by which the process may be employed. Fig. 2 is an enlarged per- 40 spective view of the die employed in the drawing process and also showing in detail the shape imparted to the drawn metal by the drawing operation.

Fig. 3 shows diagrammatically the steps 45 generally employed in the manufacture of tinsel, the size of the metal being greatly magnified.

Fig. 4 illustrates diagrammatically the steps employed in the manufacture of tinsel where a metal drawn by the process herein 50 illustrated is employed, the size of the metal being greatly magnified.

In carrying out the process, wire *c* formed 55 of copper or other non-ferrous metal, is wound upon a storage roll 1, and steel wire *s* is wound upon a storage roll 2. The capacity of the roll 2 containing the steel wire 60 may be much less than the capacity of the roll 1, the reasons for which will hereinafter appear. The copper and steel wires are

drawn together through a die 3 by means 55 of drums 4 and 5, to which the copper and steel wires are connected respectively. The drum 4 is driven by a pulley 6 and belt 7 connected to any suitable source of motive power, while the drum 5 is driven by a large 60 gear 8 meshing with a small gear 9 fastened upon the shaft 10 supporting the drum 4 and pulley 6. Due to this driving arrangement, the drum 4 is driven at a much greater speed than the drum 5 and consequently the 65 length of the copper wire drawn through the die 3 is much greater than that of the steel wire.

The copper or other non-ferrous metal wire is much softer than the steel wire and 70 when both are simultaneously drawn through the die, the steel wire will not be materially affected by the action of the die, whereas the copper wire will be formed into a substantial 75 crescent shape, as is shown in Fig. 2, the entire surface of the copper wire being hardened by contact with the sides of the die 3 and the steel wire *s*. The steel wire *s* has such a relatively slow movement through the die in comparison with the copper wire that 80 it serves as a part of the die 3 to shape the drawn copper wire. The steel wire is given a continual and gradual movement through the die to distribute the wear incident to the drawing operation along a considerable 85 length of wire.

The process just described is well adapted 90 for the manufacture of tinsel. In practice, tinsel is made by drawing copper or other non-ferrous metal wire through a die which 95 slightly reduces its cross section, and at the same time gives the drawn metal tensile strength. The metal thus drawn is flattened to produce tinsel. Fig. 4 of the drawings 100 illustrates these steps which have heretofore been employed for making tinsel, 11 representing the wire previous to being drawn, 12 the drawn and slightly reduced wire, and 13 the drawn wire flattened into tinsel. It has been found in practice that 105

when tinsel is made in this manner, the flattening of the drawn metal destroys to a considerable extent the tensile strength imparted to it by the reducing operation, this loss of tensile strength increasing proportionally to the amount of flattening the drawn wire needs in order to form it into 110 tinsel.

The process for drawing copper wire and increasing its tensile strength, which has been previously described, may be used to great advantage in the manufacture of tinsel and where so employed the metal is shaped to assume forms diagrammatically shown in Fig. 4. In this figure, 14 illustrates the undrawn copper or other non-ferrous metal, 15 shows the shape into which it is formed by the process which has been previously described, in which a steel wire is passed through the die simultaneously with the copper wire and 16 the drawn wire flattened into tinsel. The wire 15 drawn by the process previously described has a great tensile strength, and having a crescent shape, needs much less flattening to form it into tinsel than where the drawn wire has a circular cross section.

20 What is claimed is:

1. The method of working non-ferrous metals consisting in drawing a non-ferrous metal and a metal harder than the non-ferrous metal through a die together.
2. The method of working non-ferrous metals consisting in drawing a non-ferrous metal and a metal harder than the non-ferrous metal through a die together and causing one of the metals to pass through the die at a greater speed than the other.
3. The method of working non-ferrous metals consisting in drawing a non-ferrous metal and a metal harder than the non-ferrous metal through a die together and causing the non-ferrous metal to pass through the die at a greater speed than the other metal.
4. The method of working copper consisting in drawing copper and steel through a die together.
5. The method of drawing copper wire, consisting in passing copper wire and steel wire through a die together and causing the

copper wire to pass through the die at a greater speed than the steel wire.

45 6. The method of making tinsel consisting in drawing wire to give it a crescent cross section and then flattening the drawn wire.

50 7. The method of making tinsel consisting in drawing a non-ferrous metal and a hard metal through a die together to form non-ferrous wire having a crescent-shaped cross section.

55 8. The method of making tinsel consisting in drawing a non-ferrous metal and a hard metal through a die together to form a non-ferrous wire having a crescent-shaped cross section and then flattening the drawn wire.

60 9. The method of working metals consisting in drawing two metals of different degrees of hardness through a die together and causing one of the metals to pass through the die at a greater speed than the other.

65 10. The method of working metals consisting in drawing two metals of different degrees of hardness through a die together and causing the softer metal to pass through the die at a greater speed than the other metal.

70 11. The method of making tinsel consisting in drawing two metals of different degrees of hardness through a die together so as to give the softer metal a crescent-shaped cross section.

75 12. The method of making tinsel consisting in drawing two metals of different degrees of hardness through a die together so as to give the softer metal a crescent-shaped cross section and then flattening the drawn metal.

In witness whereof, we hereunto subscribe our names this 19th day of June A. D., 1919.

OLIVER C. GILBERT.  
EDGAR W. ADAMS.